

1

3,189,456

## RADIATION-SENSITIVE EMULSIONS AND ELEMENTS AND THEIR PREPARATION

Heman Dowd Hunt, Eatontown, N.J., assignor to E. I. du Pont de Nemours and Company, Wilmington, Del., a corporation of Delaware  
No Drawing. Filed June 19, 1961, Ser. No. 117,805  
2 Claims. (Cl. 96—102)

This invention relates to radiation-sensitive, silver-halide emulsions; to photographic elements embodying the same and to processes for making the emulsions. More particularly, it relates to such products and processes wherein the emulsions and elements are direct-writing, light-developable, have high speed and resolution, and have good contrast and image stability.

Radiation sensitive papers adapted for light recording, e.g., oscillographic recording, are known. These papers are commonly of the developing-out and print-out types. The developing-out type, as the name implies, requires that the exposed paper be chemically developed, fixed and washed in order to provide a stable visible image. The print-out type of paper requires no liquid development step and may or may not be stabilized and fixed. Such papers are generally much slower than those papers used in the developing-out processes and the images are unstable and have a short life. The images become masked as the background fogs or increases in density so that image detail is lost.

A third type of radiation-sensitive paper especially suitable for light-writing and oscillographic recording comprises a silver halide emulsion layer which, when exposed to a high intensity source of radiation, forms a latent image which can then be developed by exposure to diffuse daylight or artificial light of lower intensity. Such layers are faster than print-out emulsions and require no chemical development. It is this third type of direct-writing, light-developable photographic silver halide emulsion and printing material with which the present invention is concerned.

Proposed emulsions of the third type, prior to the invention of Hunt U.S. application Ser. No. 814,954, filed May 22, 1959, now abandoned, in general include silver-bromide emulsions which have incorporated therein, sulfur-containing compounds as halogen acceptors, e.g., thiourea and thio-semicarbazides. The background and image densities of layers comprising such emulsions, however, are not sufficiently stable to permit rapid access to or prolonged examination of the recorded images. It has also been proposed to make radiation-sensitive emulsions of the third type by introducing silver thiocyanate into a silver bromide emulsion. The sensitivity of this emulsion is greater than pure silver bromide emulsions containing halogen acceptors. However, such emulsions, after being light-developed, do not provide a stable image. Upon prolonged exposure to ordinary illumination, the background darkens quite rapidly which reduces the ratio between background and image densities. Also, where the development radiation contains a high proportion of ultraviolet light, subsequent exposure to such light (after light development) causes an increase in background density and rapid regression of the light-developed image. It is necessary to bathe the light-developed image in a liquid developing bath containing a silver halide solvent to intensify and preserve the contrast or ratio of background to image density of the originally light-developed image. Treatment in a conventional photographic fixing bath is also recommended.

Recently it has been found that light-developable direct-writing, radiation-sensitive elements can be made which have greatly enhanced internal latent image developability. Such elements are made by adding to a conven-

2

tionally made molten silver halide emulsion ready for coating at least 0.5 mole percent of a water-soluble stannous salt based on the silver halide in the presence of at least one water-soluble inorganic halide preferably a bromide to provide an excess of halide ions over that necessary to react with the soluble silver salts in the system. Such emulsions are disclosed in assignee's copending Hunt U.S. application Ser. No. 61,840, filed Oct. 11, 1960, Patent No. 3,033,678, May 8, 1962. Suitable elements are made according to a modification of the invention described in the Hunt application. This modification involves addition of at least 0.1 mole percent of a water-soluble, ionizable plumbous salt to stabilize the background. This modification constitutes the invention and subject matter of assignee's copending application Hunt U.S. Ser. No. 852,190, filed Nov. 12, 1959, Patent No. 3,033,682.

As disclosed in the two copending Hunt applications, the photographic elements coated with the above emulsions are quite useful in oscillographic instruments where the exposing radiation is primarily in the ultraviolet and blue regions of the spectrum. Xenon tubes and high-pressure mercury arc lamps are usually used in these instruments. Speed in oscillography is measured in inches per second of a moving spot of light and is called writing speed. For the above described elements, the writing speed is of the order of about 40,000 inches per second in a direct-writing instrument using a high-pressure mercury arc lamp.

An object of this invention is to provide new and commercially useful light-developable, direct writing, radiation-sensitive photographic silver halide emulsions, emulsion layers and elements, e.g., papers and films, embodying such layers. Another object is to provide such products which can be exposed with visible radiation as well as ultraviolet radiation. Another object is to provide such elements which have high writing speeds. A further object is to provide a simple and effective process for preparing such emulsions. Still further objects will be apparent from the following description of the invention.

The novel light-developable, direct-writing silver halide emulsions of this invention comprise a washed, light-sensitive colloid silver halide emulsion having an average grain size of 0.1 to 10 microns containing (1) 0.5 to 120 mole percent of a water soluble stannous salt, (2) a sensitizing amount of an optical sensitizing dye taken from the group consisting of cyanine, pseudocyanine, carbocyanine and merocyanine dyes capable of extending the sensitivity of a silver bromide emulsion from the normal blue region to at least one of the green, red and infrared regions of the spectrum, and having added thereto (3) at least one water-soluble halide taken from the group consisting of lithium, sodium, potassium, calcium, magnesium and ammonium chloride, bromide and iodide in an amount sufficient to provide an excess of halide ions over that necessary initially to precipitate all of the silver as silver halide. In general, there should be at least a 10% excess of halide ions present and they preferably are bromide ions. The preferred emulsions will also contain (4) 0.1 to 25 mole percent of a water-soluble inorganic plumbous salt per mole of silver. The sensitizing dye, in general, will be present in an amount from 0.1 to 0.5 millimoles per mole of silver.

According to a further aspect of the invention, the process for making the light-developable direct-writing colloid-silver halide emulsion is characterized by adding to the liquefied, washed (i.e., with water) colloid-silver halide emulsion having an average silver halide grain size in the range of 0.1 to 10 microns, the desired optical sensitizing dye, maintaining the emulsion at a temperature from 50° C. to 70° C. for a period of about 5 minutes

to about 20 minutes so that the dye is thoroughly mixed and strongly adsorbed to the silver halide grains, then adding about 0.1 to 120 mole percent, preferably about 5 to 60 mole per cent, of a water-soluble stannous salt per mole of silver halide and, if desired, 0.1 to 25 mole per cent of a water-soluble ionizable plumbous salt per mole of silver halide, and the water-soluble inorganic halide referred to above. The water-permeable silver halide colloid emulsion thus formed can be bulked up by the addition of more of the water-permeable colloid or of a different compatible water-permeable colloid. An aqueous solution can be used for this purpose. The sensitizing dye is preferably added to the emulsion from a solution in anhydrous or aqueous ethanol and the stannous and plumbous salts can be added from water, ethanol, glycerine, monethylether of ethylene glycol, or other water miscible organic solvent. In the case of hydrous salts, e.g., hydrous stannous salts, they may be added in the liquefied or molten form.

The washed silver halide emulsion used in accordance with the invention can be made by washing with water to remove soluble salts. A colloid silver halide emulsion can be made by precipitating the silver halide or mixture of silver halides in an aqueous solution containing a water-permeable organic colloid, in any conventional manner. Thus, they can be made by slowly adding an aqueous solution containing a water-soluble silver salt, e.g., silver nitrate, to an aqueous solution containing (1) a water-soluble halide or a mixture of such halides, e.g., lithium, sodium, potassium, calcium, magnesium or ammonium chloride, bromide or iodide and (2) a water-permeable organic colloid of high molecular weight and possessing protective colloid properties, preferably gelatin. In making silver bromide emulsions, it is preferable to use potassium bromide in an amount sufficient to provide an excess of 10% to 50% or more of bromide ion over that necessary to react with the silver salt, e.g., silver nitrate.

After precipitation, ripening is allowed to proceed to provide the proper grain size. The emulsions may or may not be digested, as desired, and additional water-permeable colloid added to bulk up the emulsion.

Suitable stannous salts include stannous chloride, anhydrous stannous chloride  $[SnCl_2 \cdot 2H_2O]$  and stannous sulfate. Suitable lead or plumbous salts which can be used include plumbous nitrate and plumbous acetate.

The optical sensitizing dyes referred to above preferably do not contain water-solubilizing groups in the nucleus, e.g., sulfonic or carboxylic groups and their water-soluble sodium, potassium, ammonium and amine salts because it is desirable to use dyes which are readily and strongly adsorbed to the silver halide grains. The photographic emulsions obtained in accordance with the above procedures can be coated onto a suitable base in any of the conventional manners for coating gelatino-silver halide emulsions onto paper or polymeric film base.

In processing the silver halide emulsion coated elements described above, it is only necessary after the image-forming exposure, to expose the element to ordinary artificial room light or diffuse daylight or any actinic radiation of lower intensity than the exposing light. More intense radiation may be used if the element is heated during this second step. Photodevelopment under 40-watt, white fluorescent lights at 50 foot-candles intensity has been found to be satisfactory. Higher photographic speed is obtained by the presence of optical sensitizing dyes and greater flexibility in the selection of oscillographic light sources is possible. The process of the invention is equally satisfactory when used with emulsions containing water-soluble stannous salts alone in combination with an excess of bromide ions, which are heat-stabilized after the image exposure according to the disclosure of Hunt U.S. application Ser. No. 61,840 (U.S.P. 3,033,678) or with the addition of water-soluble plumbous salts with the stannous salts and an excess of bromide ions according to the dis-

closure of Hunt U.S. application Ser. No. 852,190 (U.S.P. 3,033,682).

In the process of this invention, sequence of the addition of the various constituents to the washed colloidal silver halide emulsions is quite important. Applicant has found, which is quite surprising, that the sensitizing dye cannot be successfully added after the water-soluble stannous and plumbous salts have been added, because the latter have an adverse effect on the sensitizing action of the dye if they are added later.

The photographic elements of this invention embodying the novel dye-sensitized, light-developable, direct-writing silver halide emulsions can be subjected to an image-forming exposure by means of radiation, the spectral composition of which preferably includes radiation in the region of inherent sensitivity of the silver halide emulsion and also radiation in the region of extra response of said emulsion conferred by addition of the optical sensitizing dye. The exposure time may be the same as described in the patent applications referred to above and range from 0.01 or less to 10,000 microseconds depending on the intensity of the exposing light. After exposure, the element is either subjected to heat and light or higher intensity or to white light of about 50 foot-candles for photodevelopment. Without heat, the photodevelopment radiation must be of less intensity than the exposing light.

In the detailed illustrative examples which follow, the coated elements were tested by using a Mark III Edgerton, Germenshausen and Grier, Inc., electronic flash sensitometer similar to that described by Wyckoff and Edgerton, Journal of the Society of Motion Picture and Television Engineers 66, 474 (1957). This instrument contains a xenon discharge tube as a source of radiation and the exposure time was  $10^{-5}$  seconds. The sensitometer was modulated with a  $\sqrt{2}$  step tablet of 21 steps ranging in density from 0.05 to 3.05. The latent image formed was photodeveloped by exposing the element to white light for a period of several minutes to obtain maximum image density. With this type of light-development, a much more stable image is obtained. Light-development by first heating and then exposing to a higher intensity light source can result in a readable image in about one second or less, with only a slight increase in background density.

The present invention will be further illustrated by, but is not intended to be limited to, the following detailed examples.

#### Example I

A gelatino-silver chlorobromide emulsion was made in the following manner. To an approximately 1% aqueous gelatin solution containing 1.5 moles of potassium chloride and .075 mole of hydrochloric acid there was added over a period of 25 minutes at a temperature of 140° F. one liter of 1.5 molar solution of silver nitrate. The emulsion was held for 5 minutes and there was then added 160 mole percent of potassium bromide based on the silver. The emulsion was ripened for 40 minutes at 140° F. and cooled. The emulsion was washed by coagulation and redispersed in the manner described in Example I of Moede U.S. 2,772,165. The gelatin concentration was raised to approximately 6.5% during which time the temperature was raised to and held at 130° F. At this point, 150 milligrams of the dye: 5,5'-dimethyl 3,3',9-triethyl benzoselenazole carbocyanine iodide was added from a 1:1000 methanolic solution. The preparation of this dye is disclosed in U.S. Patent 1,990,681. The emulsion was held at 130° F. for five minutes and then there was added an aqueous solution of plumbous nitrate in an amount to provide one mole percent of lead based on the silver halide. Potassium bromide was added to give an excess of 30 mole percent of bromide ions based on the silver halide. The emulsion was again held for five minutes at 130° F. and 10 mole percent of stannous chloride was added from a 57% aqueous solution. The emulsion was

held for five minutes at 130° F. and then cooled to 95° F. Various coating aids including a hardener were added and the emulsion was coated to give a coating weight equivalent to 30 milligrams of silver nitrate per square decimeter. The coated emulsion was dried in a conventional manner. The emulsion was exposed in the sensitometer described above to white light, blue light by means of a Wratten #47 filter, green light by means of a Wratten #61 filter, and to red light by means of a Wratten #29 filter. Under the influence of the  $10^{-5}$  second flash exposure in the sensitometer, the following results were obtained which are given as the number of steps made visible through the  $\sqrt{2}$  step wedge. The photodevelopment step consisted of exposure for 30 minutes under 40-watt white fluorescent lights at 50 foot-candles intensity. The letters W, B, G, and R indicate white, blue, green and red, respectively. The term  $D_{21}$  indicates the density of step 21 of the wedge for a white light exposure after 30 minute photodevelopment. The term  $\Delta$  indicates the differences between fog or background density and image density obtained through step 21 of the 2 step wedge. A control containing no sensitizing dye was also exposed for comparison.

|              | W  | B  | G     | R     | $D_{21}$ | Fog | $\Delta$ |
|--------------|----|----|-------|-------|----------|-----|----------|
| Test.....    | 17 | 12 | 8     | 13    | .51      | .17 | .34      |
| Control..... | 17 | 14 | ----- | ----- | .48      | .16 | .32      |

#### Example II

Example I was repeated except that 150 milligrams of 3,3'-diethyl-9-methyl-benzothiazole carbocyanine p-toluene sulfonate was added in place of the dye of Example I. This dye is described by Hamer in J.C.S. 1928, pages 3160-3163. All operations in the preparation, coating, drying and testing were carried out in the same manner as described in Example I with the following results.

|              | W  | B  | G     | R     | $D_{21}$ | Fog | $\Delta$ |
|--------------|----|----|-------|-------|----------|-----|----------|
| Test.....    | 18 | 12 | 12    | 7     | .55      | .21 | .34      |
| Control..... | 17 | 14 | ----- | ----- | .48      | .16 | .32      |

#### Example III

Example I was repeated except that in place of the optical sensitizing dye of that example there was added 150 milligrams of the dye: 5,5'-dibromo-3,3'-diethyl-9-methyl benzothiazole carbocyanine p-toluene sulfonate. All other conditions and operations remained the same. The exposure results are as follows:

|              | W  | B  | G     | R     | $D_{21}$ | Fog | $\Delta$ |
|--------------|----|----|-------|-------|----------|-----|----------|
| Test.....    | 17 | 12 | 9     | 9     | .51      | .23 | .28      |
| Control..... | 17 | 14 | ----- | ----- | .48      | .16 | .32      |

#### Example IV

Example I was repeated using in place of the optical sensitizing dye of that example, 150 milligrams of the dye: 5,5'-trimethyl-3,3'-diethyl benzothiazole carbocyanine iodide. All other conditions and operations remained the same. The exposure results are as follows:

|              | W  | B  | G     | R     | $D_{21}$ | Fog | $\Delta$ |
|--------------|----|----|-------|-------|----------|-----|----------|
| Test.....    | 17 | 13 | 11    | 9     | .51      | .19 | .32      |
| Control..... | 17 | 14 | ----- | ----- | .48      | .16 | .32      |

#### Example V

Example I was repeated using 150 milligrams of the dye: 5,5'-diphenyl-9-methyl-3,3'-diethyl benzoxazole car-

bocyanine iodide. All other conditions and operations remained the same. The exposure results are as follows:

|              | W  | B  | G     | R     | $D_{21}$ | Fog | $\Delta$ |
|--------------|----|----|-------|-------|----------|-----|----------|
| Test.....    | 19 | 13 | 14    | ----- | .48      | .17 | .31      |
| Control..... | 17 | 14 | ----- | ----- | .48      | .16 | .32      |

#### Example VI

Example I was repeated using 150 milligrams of the dye: 5,5'-dimethyl-3,3'-triethyl benzothiazole carbocyanine iodide. All other conditions and operations remained the same. The exposure results are as follows:

|              | W  | B  | G     | R     | $D_{21}$ | Fog | $\Delta$ |
|--------------|----|----|-------|-------|----------|-----|----------|
| Test.....    | 17 | 12 | 8     | 9     | .55      | .20 | .35      |
| Control..... | 17 | 14 | ----- | ----- | .48      | .16 | .32      |

#### Example VII

Example I was repeated using 150 milligrams of the dye: 5,5'-dimethyl-9-phenyl 3,3'-diethyl benzothiazole carbocyanine iodide. All other conditions and operations remained the same. The exposure results are as follows:

|              | W  | B  | G     | R     | $D_{21}$ | Fog | $\Delta$ |
|--------------|----|----|-------|-------|----------|-----|----------|
| Test.....    | 16 | 12 | 3     | 5     | .53      | .22 | .31      |
| Control..... | 17 | 14 | ----- | ----- | .48      | .16 | .32      |

#### Example VIII

Example I was repeated with plumbous nitrate being omitted. All other additions, operations in preparation, coating, drying and testing were carried out in the same manner as described in Example I with the following results:

|              | W  | B     | G     | R     | $D_{21}$ | Fog | $\Delta$ |
|--------------|----|-------|-------|-------|----------|-----|----------|
| Test.....    | 18 | ----- | 8     | 13    | .58      | .30 | .28      |
| Control..... | 17 | 14    | ----- | ----- | .48      | .16 | .32      |

While stannous chloride can be used in aqueous solutions, the solutions tend to become cloudy although this characteristic does not appear to interfere with its activity in the system. To overcome the cloudiness the stannous chloride may be dissolved in glycerine or sorbital which provides a convenient means of adding an anticurl agent to the emulsion which is especially desirable in coatings on paper. Other stannous salts may be used such as, for example, stannous sulfate.

The optical sensitization of emulsions of this invention is not affected by the presence of relatively high quantities of stannous salts. In this respect the presence of stannous salts is not critical. This is considered to be an advantageous and novel feature because since the stannous compounds have such a profound effect on the silver halide, it would logically be assumed that its presence would interfere with the adsorption of the sensitizing dye on the silver halide grain. This would be true if the dyes were added at the same time or after the tin and lead salts were added. Additional suitable sensitizing dyes which can be used in place of those in the examples and modifications of the invention include the merocyanines disclosed in Kendall U.S.P. 2,272,163 and the selenopseudocyanines disclosed in Dieterle et al. U.S.P. 2,310,339.

Where it is desired, other halides or combinations of halides may be used to form the silver halide grains. For example, pure silver chloride, chlorobromide or iodobromide may be used. Where soluble chloride salts are used, it is desirable, because of solubility product differences, to form the silver halide grains of desired concen-

tration before the addition of the excess bromide ions. The operative association of lead salts with excess bromide ions is advantageous in that the washing step may be eliminated if desired.

In place of the gelatin binding agent used in the foregoing examples, there may be substituted other natural or synthetic water-permeable organic binding agents. Such agents include water-soluble or -permeable polyvinyl alcohol and its derivatives, e.g., partially hydrolyzed polyvinyl acetates, polyvinyl ethers and acetals containing a large number of extralinear  $-\text{CH}_2\text{OH}-$  groups; hydrolyzed interpolymers of vinyl acetate and unsaturated addition polymerization compounds, for example, maleic anhydride, acrylic and methacrylic acid esters and amines and styrene. Suitable colloids of the last mentioned type are disclosed in U.S. Patents 2,276,322, 2,276,323 and 2,397,866. The useful polyvinyl acetals include polyvinyl acetaldehyde, polyvinyl butyraldehyde and polyvinyl sodium o-sulfonylbenzaldehyde. Other useful colloid binding agents include the poly-N-vinyl lactams of Bolton U.S. Patent 2,495,918. These compounds include polyvinyl pyrrolidone. N-acrylamido alkyl betaines and copolymers thereof are described in Shacklett, U.S. Patent 2,833,650.

As disclosed above, the dye-sensitized emulsions of this invention can be coated on any suitable support, e.g., sized or unsized paper, or paper substitutes made from non-cellulosic fibers, or a polymeric film composed of a cellulose ester including cellulose acetate, cellulose propionate and cellulose acetate/butyrate or a superpolymer such as polyvinyl chloride co vinyl acetate; a polyvinyl acetal, e.g., a formal or acetaldehyde acetal; polystyrene; polyamide, e.g., polyhexamethylene adipamide or a polyester, e.g., polyethylene terephthalate and polyethylene terephthalate/isophthalate. The vinylidene chloride copolymer-coated oriented flexible polyester films of Alles et al. U.S. Patent 2,627,088 and Alles U.S. 2,779,684 are quite suitable supports. The various film bases may, if desired, contain a suitable white or other colored opacifying agent.

An advantage of the invention is that the optical sensitization of the light-developable, direct-writing, colloid-silver halide emulsion layers is not affected by the presence of the relatively large quantities of stannous salts. This is quite surprising and is probably due to the fact that the dye is added first, as stannous compounds ordinarily have a profound effect on the silver halide grain and it would logically be assumed that its presence would interfere with adsorption of the sensitizing dye on the silver halide grains.

The radiation-sensitive elements of this invention, in addition to being extremely convenient to use because of the elimination of wet-processing, also offer the outstanding advantage of higher photographic speed or permits the use of lamps weak in blue light because of their increased response in the infrared and visible regions of the spectrum. Dry processing allows the operator to see and use a print image rapidly after recording. Seismology, electrocardiograms, photocopying, X-recording and studio

proof papers are fields in addition to oscillography where the novel light-sensitive elements of this invention can be used.

I claim:

- 5 1. A process for making light-developable, direct-writing colloid-silver halide emulsion characterized by adding to the liquefied, washed colloid-silver halide emulsion having an average silver halide grain size in the range of 0.1 to 10 microns, an optical sensitizing dye selected from the group consisting of cyanine, pseudocyanine, carbocyanine and merocyanine dyes capable of extending the sensitivity of a silver bromide emulsion from the normal blue region to at least one of the green, red and infrared regions of the spectrum, maintaining the emulsion at a 15 temperature of from 50° C. to 70° C. for a period of about 5 minutes to about 20 minutes so that the dye is thoroughly mixed and strongly adsorbed to the silver halide grains, then adding about 0.1 to 120 mole percent of a water-soluble stannous salt per mole of silver halide and 20 a water-soluble halide.
2. A process for making light-developable, direct-writing colloid-silver halide emulsion characterized by adding to the liquefied, washed colloid-silver halide emulsion having an average silver halide grain size in the range 25 of 0.1 to 10 microns, an optical sensitizing dye selected from the group consisting of cyanine, pseudocyanine, carbocyanine and merocyanine dyes capable of extending the sensitivity of a silver bromide emulsion from the normal blue region to at least one of the green, red and infrared regions of the spectrum, maintaining the emulsion at a 30 temperature of from 50° C. to 70° C. for a period of about 5 minutes to about 20 minutes so that the dye is thoroughly mixed and strongly adsorbed to the silver halide grains, then adding about 0.1 to 120 mole percent of a water-soluble stannous salt and about 0.1 to 25 mole percent of a water-soluble plumbous salt, per mole of silver halide, and a water-soluble halide.

#### References Cited by the Examiner

| UNITED STATES PATENTS |      |                 |          |
|-----------------------|------|-----------------|----------|
| 2,005,837             | 6/35 | Arens           | 96—64    |
| 2,323,187             | 6/43 | Arens et al.    | 96—64    |
| 2,497,876             | 2/50 | Fallesen et al. | 96—64    |
| 2,541,472             | 2/51 | Kendall et al.  | 96—64    |
| 2,756,148             | 7/56 | MacWilliam      | 96—102   |
| 2,993,893             | 7/61 | Hunt            | 96—102 X |
| 3,033,678             | 5/62 | Hunt            | 96—94 X  |
| 3,033,682             | 5/62 | Hunt            | 96—94 X  |

#### FOREIGN PATENTS

|         |      |                |
|---------|------|----------------|
| 485,609 | 5/38 | Great Britain. |
|---------|------|----------------|

#### OTHER REFERENCES

|    |                                                                                                                       |
|----|-----------------------------------------------------------------------------------------------------------------------|
| 55 | Classification Bulletin of the U.S. Patent Office No. 422, Class 96, Photographic Chemistry, Processes and Materials. |
|----|-----------------------------------------------------------------------------------------------------------------------|

NORMAN G. TORCHIN, Primary Examiner.

60 HAROLD N. BURSTEIN, Examiner.